

May 6, 1941.

S. E. DIESCHER

2,241,083

METHOD OF MAKING UPSET SEAMLESS TUBING

Filed Nov. 7, 1938

3 Sheets-Sheet 1



WITNESSES  
A. B. Wallace.  
E. O. Johns

BY

INVENTOR.  
Samuel E. Diescher  
by Brown, Critchlow & Lib

his ATTORNEYS.

May 6, 1941.

S. E. DIESCHER

2,241,083

METHOD OF MAKING UPSET SEAMLESS TUBING

Filed Nov. 7, 1938

3 Sheets-Sheet 2



BY

INVENTOR.  
Samuel E. Diescher  
By Brown, Crittenden & Hulc

his ATTORNEYS.

May 6, 1941.

S. E. DIESCHER

2,241,083

METHOD OF MAKING UPSET SEAMLESS TUBING

Filed Nov. 7, 1938

3 Sheets-Sheet 3



INVENTOR

Samuel E. Diescher  
By Brown, Crittenden & Fitch

his ATTORNEYS.

## UNITED STATES PATENT OFFICE

2,241,083

## METHOD OF MAKING UPSET SEAMLESS TUBING

Samuel E. Diescher, Pittsburgh, Pa., assignor to  
Diescher Tube Mills, Inc., Pittsburgh, Pa., a  
corporation of Delaware

Application November 7, 1938, Serial No. 239,211

7 Claims. (Cl. 80—62)

This invention relates to the manufacture of seamless tubing having one or more portions of it provided with a wall thickness greater than normal, or, in other words, having what is conventionally known as one or more upsets. Throughout this specification, and in the claims "upset" is used to designate that portion of a tube whose wall is thicker than the normal wall thickness of the tube.

Tubing having upset ends is used for various purposes, but perhaps most extensively in the oil and gas fields for drill pipe, well tubing and well casing. As now manufactured, the end of a tube, whether of the seamless or welded type, is first heated and then subjected in suitable dies to compression in a direction parallel to the axis of the tube to upset or thicken the metal. This is a hot work operation that is performed subsequent to the production of tubes, and accordingly adds materially to their cost of manufacture. Furthermore, in such operations it is difficult, if not impossible, so to upset the ends of tubes that the transition from the thickened to the normal wall is of a sufficiently gradual slope fully to meet many requirements of service. For example, when conventionally formed upset tubing is subjected to vibration it is liable to break in the region of its transition from its upset to its normal wall thickness by reason of the insufficient slope of wall thickness in such region. Also, the upsets that can readily be formed in the conventional manner just explained are so limited in length that the upset ends of the tubes cannot be repeatedly cut back for rethreading, as is frequently desirable in the repeated use of oil and gas country goods. For longer upsets or upsets made in lighter wall product more than one such upsetting operation is required, and, in the lightest wall product that can be made by hot working, upsetting by the usual method may be regarded as being commercially impossible.

While upset tubing is now made in the manner just explained, the prior art contains several suggestions that upsets be formed in the course of production of tubing, and particularly in the manufacture of seamless tubing by the swaging process. According to these suggestions, swaging mandrels are provided with portions which are of smaller than normal diameter and on which upsets or thickened portions are swaged. Because such tubes are formed in closed passes they stick tightly upon the mandrels. This requires the upsetting to be performed in stages, each preceded by a partial extraction of the

mandrel which introduces a time consuming additional and costly operation.

The objects of the present invention are to provide a method of manufacturing upset seamless tubing in which the upsets can be made of any desired length, at the ends or in any desired positions throughout the length of the tubing, with any desired slope in the transition from the upsets to the normal wall thickness, and without 10 performing any manufacturing step in addition to those required for the production of tubing having uniform wall thickness from end to end except when the tubing is produced with relatively thick upsets.

15 In my United States Patent No. 1,870,209 there is disclosed a method of reducing the wall thickness and elongating a tubular blank, according to which, in the manner therein specifically disclosed, a tubular blank or work piece is cross-rolled on a cylindrical mandrel of the same cross-section throughout its working extent. The helically acting cross-rolls uniformly reduce the wall thickness of the blank and cause it to bulge laterally away from the mandrel between such rolls, and feed the blank and the mandrel forward. Between the cross-rolls the lateral bulging of the blank is limited, the peripheral flow of the metal is diverted longitudinally, and the metal of the blank is pulled forwardly by a pair 25 of guide discs that are driven at a peripheral speed in excess of the speed of longitudinal movement of the blank effected by the cross-rolls.

30 My present invention is predicated primarily upon my discovery that its stated objects can be attained during the elongating and wall reducing of tubular blanks according to the method of my aforesaid patent by effecting the cross-rolling on a mandrel which has a normal-diameter cylindrical portion for determining the normal wall thickness of the elongated tubing, and which has a smaller-diameter portion for producing an upset, or, in other words, a greater than normal wall thickness. I have found that by properly 35 coordinating controllable elements and factors of the mill and method disclosed in my aforesaid patent, a seamless tube can be provided with normal upsets at one or both of its ends and also at any desired intermediate point or points throughout its length without performing any 40 operation in addition to those required for the production of a like tube of uniform wall thickness from end to end. When it is desired to similarly provide a tube with one or more relatively thick, as distinguished from normal, upsets an additional procedural step of a simple

and inexpensive character is ordinarily required.

The invention will be explained with reference to the accompanying drawings in which it is diagrammatically illustrated, and of which Fig. 1 is a vertical central sectional view through a mill, similar to that disclosed in my aforesaid patent, the elements of the mill being formed and co-ordinated to elongate a tubular blank and simultaneously to provide its ends with upsets; Fig. 2 a central sectional view through a mandrel stripper in the operation of removing a mandrel from a tube after the completion of an elongating operation in which the ends of the tube have simultaneously been provided with normal upsets; Fig. 3 a view similar to Fig. 2 showing the stripper in the operation of removing a mandrel on which a tube has been elongated and simultaneously provided with normal upsets intermediate of its ends; Fig. 4 a vertical longitudinal central view of an apparatus for removing a mandrel from a tube that has been elongated and simultaneously provided with relatively thick end upsets; Fig. 5 a detailed view, partly in longitudinal central section, of the end of a specially formed mandrel; Fig. 6 a longitudinal central sectional view of a portion of an expander for converting interior to exterior upsets; Fig. 7 an end view, partly in central longitudinal section, of the end of a tube provided with an exterior end upset; Figs. 8 and 9 elevations of the side and end, respectively, of a rotating expanding tool such as used in the expander of Fig. 6; and Fig. 10 a vertical longitudinal central sectional view of a reciprocating expander operating upon the end of a tube initially provided with an interior upset.

In the practice of my invention in its applicability to the elongating of tubular blanks and simultaneously providing them with normal end upsets, it is first necessary to provide suitable mandrels, such as illustrated in Fig. 2. Each such mandrel has a normal-diameter cylindrical portion 2 which cooperates with helically acting reducing rolls to determine the normal wall thickness of the resultant tube, and is provided at its front and rear ends with smaller-diameter portions 3 and 4, respectively, which similarly co-operate with such rolls to produce upsets at the ends of tubes. Although it is not essential, it is preferred to have the rear small-diameter portion 4 of greater length than the forward portion 3. Between its end and intermediate portions the mandrel is provided with tapered sections 5, the extent of which is determined largely from the slope of transition that is desired from the upsets to the normal wall thickness of a tube. This special forming of mandrels involves merely a machining operation that adds little, if any, to the cost of production of the tubes.

A mandrel such as just described is placed within a thick-wall tubular blank which may be, and preferably is, produced by piercing a solid billet, although other tubular blanks may be used. Because the extent of the forward end upset of an elongated tube depends upon the length of the forward end of the blank that is reduced between the cross rolls and the smaller-diameter portion 3 of the mandrel, it is desirable definitely to position the end of the mandrel with relation to that of the blank. This may be done in the manner disclosed in United States Patent No. 1,964,507 to A. P. Diescher, and shown particularly in Fig. 4 thereof, by positioning the forward end of the blank against a removable stop and moving the mandrel through the blank until

its forward end engages another removable stop placed at definite, although variable, distance ahead of the first-mentioned stop.

With a heated blank and a mandrel thus telescopically assembled, they are passed through a cross roll reducing mill of the type illustrated in Fig. 1, the working elements of the mill having first been suitably adjusted to obtain the desired result as will presently be explained. This mill comprises a pair of oppositely disposed helically acting rolls 6, which may be of general barrel-shape type, as illustrated, although they may be of any other desired type or form such as conical or disc. When barrel-shaped cross rolls are used their axes are inclined to each other and to the line of feed of a blank between them. Disposed between the cross rolls, and on opposite sides of the pass between them, there are surfaces that bear on the blank and move in the direction of its longitudinal extent. These surfaces are preferably the grooved peripheries of a pair of guide discs 7 which are driven at a peripheral speed materially in excess of that of the longitudinal movement of the blank effected by the helically acting cross rolls. In adjusting the mill the cross rolls are so positioned laterally from the center line of the pass that at the throat, or most constricted portion, of the pass they are spaced apart a distance equal to the diameter of the large-diameter portion 2 of the mandrel, plus twice the thickness of the normal wall portion of a desired tube. This spacing with relation to the different diameter portions of the mandrel determines both the normal and the upset wall thicknesses of the tube. The guide discs are so positioned above and below the center line of the pass that their peripheries, in the throat of the pass, are spaced at the optimum permissible distance from the mandrel in excess of the spacing of the cross rolls. In thus positioning the guide discs, due consideration must be given to preserving their functions of diverting longitudinally the peripheral flow of the metal, limiting the bulging of the blank between the cross rolls and away from the mandrel, and pulling the blank forward in the pass.

With the cross rolls and guide discs thus positioned, and with the forward ends of the blank and mandrel relatively positioned in the manner explained above, the blank and mandrel are fed forwardly in the line of pass of the mill until the front end of the mandrel is in the pass and the front end of the blank is engaged by the cross rolls. The wall thickness of the forward end of the blank is first reduced between the cross rolls and the front smaller-diameter portion 3 of the mandrel to determine the wall thickness of the forward end upset of the resulting tube. As the operation proceeds, the cross rolls act successively upon the portion of the blank between them and the tapered section 5 to determine the slope of transition from the upset to the normal wall thickness, then upon the portion of the blank between them and the normal-diameter portion 2 of the mandrel to determine the normal wall thickness of the tube, then upon the portion of the blank between them and the rear tapered section 5 of the mandrel to determine the slope of transition, and finally upon the portion of the blank between them and the rear small-diameter portion 4 of the mandrel to determine the rear end upset. As shown in Fig. 2, the resulting tube has a forward end upset 10, an intermediate portion 11 of normal wall thickness, a rear end upset 12, and sloping transition sections 13 and

14 between the upset ends 10 and 12, respectively, and the normal wall portion 11.

In thus elongating a tubular blank and simultaneously providing the ends of the resulting tubes with upsets, the metal of the blank ovals or bulges outwardly against the guide discs 7 which are driven at such peripheral speed that the elongated portion of the tube moves longitudinally at a more rapid rate than does the mandrel. Accordingly, at the end of a tube-forming operation the forward end of the mandrel normally lies within the forward end of the tube, as shown in Fig. 2. This increase of rate of longitudinal movement of the forward end of the tube is effected primarily during the elongation of the normal wall portion of the tube because of the greater reduction in wall thickness then being made, there being less and in some cases no differences, in rate of movements during the formation of the upsets 10 and 12. Because of this and of the ovality created while being rolled there is no binding of the rear upset end 12 of the tube upon the mandrel while it is being formed, regardless of the wall thickness of such upset. Should the upset be of normal thickness the ovality created in the rolling thereof will suffice to provide clearance between the bore of the upset and the body of the mandrel and thus avoid any possibility of binding, and should the upset be of heavy thickness there will be so little difference between the forward speed of the mandrel and of the upset portion as to permit what ovality that does occur to suffice for the little forward clearance that may be needed.

An important factor involved in the forming of normal upsets in the practice of this invention is that the relative spacings of the guide discs and of the cross rolls, and the relation between the diameters of the normal-diameter portion 2 and the smaller-diameter end portions 3 and 4 of the mandrel are such that the interior circumference of the upsets is greater than the circumference of the normal-diameter portion of the mandrel. The result of this coordination of the several elements of the mill is that the mandrel can be freely removed from the formed tube. This may be done in the manner illustrated in Fig. 2 by engaging the rear end of the mandrel between a pair of yieldingly mounted pinch rolls 15 which are driven to move the mandrel outwardly, and by abutting the end of the tube against a stripping collar 16. This mandrel extractor is used in removing mandrels from tubes having uniform wall thickness from end to end when they are produced according to the method disclosed in my aforesaid Patent No. 1,870,209. Accordingly, in the practice of my present invention seamless tubes having normal end interior upsets are produced without any procedural step in addition to those required in a production of such tubing having uniform wall thickness from end to end. Reference has been made to the difference in rate of longitudinal movements from the forward end of a tube and a mandrel on which it is formed. This difference in rate is substantially uniform for a given setting and driving of the mill and for a given mandrel size when used to produce end upset tubing from tubular blanks of uniform size. Accordingly, successively formed tubes have their end upsets uniformly spaced apart.

By way of example, and not of limitation, the following specific data are given to illustrate the construction and positioning of mill elements, including the mandrel, that may be used in the

practice of my invention in elongating tubular blanks and simultaneously providing them with normal end upsets in the manner explained above. The mandrel may have a normal diameter portion 20 feet 6 inches in length and 2.41 inches in diameter, and have at each end, beyond its 20 feet 6 inches normal diameter portion, a reduced portion of 2.19 inches in diameter, and the tubular pierced blanks may have an outside diameter of  $3\frac{1}{8}$  inches, a wall thickness of 0.38 of an inch, and may be 14 feet 7 inches long. With the cross rolls spaced 2.78 inches from each other at the throat of the pass, and the bottoms of the peripheral grooves of the guide discs spaced 3.10 inches from each other at the throat of the pass, the blanks will become elongated to tubes approximately 30 feet long,  $3\frac{1}{8}$  inches outside diameter from end to end, 0.185 of an inch normal wall thickness, and 0.295 of an inch wall thickness at the upset ends. The interior circumference of the end upsets will be greater than the circumference of the normal-diameter portion of the mandrel, so that the resulting tubes can readily be stripped from the mandrel in the manner shown in Fig. 2.

In the practice of the invention, tubes may be provided with one or more interior upsets intermediate of their ends by following the same procedure that has thus far been explained, except for the construction of the mandrel, which, as shown in Fig. 3, is formed to have a plurality of normal-diameter portions 20 at its ends and intermediate thereof, and a plurality of small diameter portions 21 intermediate of its ends. Tubes elongated on such mandrels have normal wall thickness sections 22 which are interrupted by upsets 23 at desired positions along their length. Because the interior circumference of the upsets 23 is larger than the circumference of the normal diameter portions 20 of the mandrel, the resulting tubes may readily be stripped from the mandrel in the manner shown in Fig. 3 and explained with reference to Fig. 2.

By way of further example, and not of limitation, the following specific data are given to illustrate the construction and positioning of mill elements, including the mandrel, that have been successfully used in the practice of my invention in elongating tubular blanks and simultaneously providing them with normal intermediate upsets of the character illustrated in Fig. 3. The mandrel has a normal-diameter portion 1.70 inches in diameter, and six smaller-diameter portions 1.56 inches in diameter. The tubular pierced blanks were 103.5 inches in length having an outside diameter of  $2\frac{1}{4}$  inches and a wall thickness of 0.295 of an inch. These blanks were elongated and sized into tubes averaging 14 feet 3 inches in length having an outside diameter of 2.35 inches, a normal wall thickness of 0.20 of an inch, and internal upsets of 0.27 of an inch in thickness. In making the upset tubes just described the main or cross rolls were spaced 2.10 inches and the guide discs 2.37 inches apart.

Tubes having upsets intermediate of their ends may advantageously be used in the manufacture of upset tubular articles in multiples, wherein the upsets are located at points where greater strength is required. Such tubes may be provided with an upset at one or both of their ends, and, in the production of tubes having no intermediate upsets, upsets may be formed at only one of their ends if desired.

By way of further example and not of limitation, the following specific data are given to ill-

lustrate the construction and positioning of mill elements, including the mandrel, that have been used in the practice of my invention in elongating tubular blanks and simultaneously providing them with very long end upsets as well as very long intermediate upsets. The mandrel had a normal diameter of 1.590 inches. It was turned down to 1.470 inches at the ends, as well as at two stations therebetween, in a manner as to provide three portions of the mandrel, each 24½ inches long, of normal diameter, and intermediate of these to provide two portions, each 22 inches long of reduced diameter, namely 1.470 inches. The intermediate tapers were 1.00 inch long. On this mandrel tubes 2 inches in diameter and 16 feet 1 inch long were rolled, having 0.240 inch of wall at 20 inches of length at their two end upsets and also at 27 inches of length at their two intermediate upsets. The three remaining portions, intermediate of the upsets, were each 33 inches long and were of 0.187 inch, or of normal wall thickness except at the transition tapers. These articles were rolled with the same ease as would have been the case were the mandrel of uniform diameter and the product of uniform wall thickness. In this case the main rolls were spaced 1.964 inches apart and the guide discs were 2.25 inches apart. The pierced shells used were 2.50 inches in diameter, 0.325 inch in wall thickness and 105 inches long.

The invention has been thus far explained in its applicability to the production of tubing having end and intermediate upsets of a normal character, as distinguished from relatively thick upset which are sometimes required. In the practice of my invention one or both ends of tubes may be provided with relatively thick upsets with no change in the elongating procedure except that the smaller-diameter end portions of the mandrels are, with the relation to their normal-diameter portions, reduced more in size than in mandrels used for producing normal upsets. One difference between an elongated tube provided at both ends with relatively thick rather than normal upsets is that in the former the interior circumferences of the upsets are smaller than the normal-diameter portion of the mandrels, as a result of which the mandrel on which each tube is formed is entrapped by the upsets. Another difference is that the outside diameter of relatively thick upset ends is slightly less than that of the normal wall thickness portion of the tube. This second difference arises from the fact that in the production of relatively thick end upsets the relatively small reduction in wall thickness of the portions of the tubular blank that form the upsets does not cause the metal to bulge laterally or oval against the guide discs to an extent sufficient to expand the circumference of the upsets to that of the normal wall thickness portion of the blank which is given a materially greater reduction by the cross rolls.

To remove a thus entrapped mandrel from a tube that has been provided with relatively thick end upsets, it is preferable to use a pusher mechanism, such as illustrated in Fig. 4, than the pinch rolls of Figs. 2 and 3, because a greater and more positive force can be applied by the pusher mechanism. As shown in Fig. 4, the pusher comprises a ram 25 attached to a cross-head 26 which is connected to the end of a piston rod 27 adapted to be reciprocated by a compressed air or other form of pressure fluid cylinder 28. In removing a mandrel by this pusher, the forward end of ram 25 may be centered in

the trailing end of the mandrel which projects from a finished tube, and the fluid pressure cylinder actuated to push the mandrel out of the tube, the end of which is engaged by a stripping collar 29. During this operation the upset at the end of the tube, which at this stage is still hot and readily deformable and which abuts against collar 29, is expanded by the tapered section of the mandrel between its normal and smaller-diameter portions. This leaves the outside diameters of the upsets of different size, the upset through which the mandrel has been removed being larger than that at the other end of the tube. However, this difference in the outside diameters of the upsets, and the difference, explained above, between the outside diameters of the upsets and normal wall portion of the tube, are not prejudicial because the tube may readily be brought to uniform diameter from end to end by passing it through sizing rolls or a sink mill as is customarily done subsequent to the production of tubes having uniform wall thickness throughout.

If at the completion of the mandrel-removing operation it is desired to have both of the end upsets of the same diameter, the pusher may be given a short stroke sufficient only to cause the mandrel to expand one upset, and the tube and its contained mandrel may then be transferred laterally to position it in line with a second similar pusher mechanism constructed to engage the other end of the mandrel and push it through the previously unexpanded upset and entirely out of the tube. If desired, the tube may then be passed through a sizing or sink mill as explained above, or its upset ends may be further expanded in a manner hereinafter described, or it may be treated in any other desired way.

To resist wear on the tapered sections of a mandrel while it is moved in the manner just explained to expand relatively thick upsets in the removal of the mandrel from tubes, such sections may, as shown in Fig. 5, be provided with heat and wear-resisting collars 30. When thus formed, the normal-diameter portion of the mandrel may consist of a cylindrical rod 31, and each smaller-diameter end portion may consist of a short rod 32 provided with an offset 33 to receive a collar 30 and with a threaded end 34 adapted to be screwed into the end of rod 31.

Although the production of tubes having relatively thick upsets requires a manufacturing step or steps in addition to those required for the production of tubing having uniform wall thickness from end to end, nevertheless no loss of operating time occurs because the additional step or steps are performed immediately after the elongating of each upset tube and in less time than required for the elongation.

In providing tubes with upsets according to this invention, all the upsets are initially of the interior type, by which is meant that the increased wall thickness of the upsets contracts the bore of the normal wall thickness portion of the tube. However, the interior upset ends of the tube can readily be converted into exterior upsets by merely expanding the ends, whether the upsets are of the normal or the relatively thick type. While in some cases this may be done on the original heat of the metal, to prevent the metal from becoming too cool to be readily expanded without impairing it, the tubes may, in their passage from the mandrel extractor to the expander, be passed through a heating furnace.

Both upset ends of a tube may be simultaneously expanded by a rotary expander such as

illustrated in Fig. 6. To do this the ends of a heated tube, and their intermediate portions as far as may be necessary, are engaged by clamps 40 which hold them in alignment with spinning heads 41, each of which is attached to or is formed on the end of a spindle 42 adapted to be rotated by a motor 43. As shown particularly in Figs. 8 and 9, spinning head 41 has a frustum-like portion 44 which effects the expanding of an upset and a cylindrical portion 45 which removes any scores that may occur during such expanding. Spindle 42 is provided centrally with a bore 46 which is closed at its outer end and through which, and radial spindle ports 47, steam or a combustible gas or lubricant is led to the face of the spindle to facilitate the spinning or expanding operation and to cool the spinning tool and also to remove scale that may accumulate at the tool. The spinning tool and its driving motor are mounted upon a table 50 which is slidably supported on a platen 51 and is engaged by a feed screw 52 rotatably mounted on the platen and adapted to be driven by a motor 53 through a worm shaft 54 and a worm gear 55. The platen 51 is slidably mounted upon a table 56 to properly position the spinning tool for operation upon tubes of different lengths. As the spinning head 41 is rotated by the motor 43, screw 52 is driven by motor 53 to feed the head through the upset end of the tube until the entire upset, including the adjoining transition portion of the tube, is so expanded that its inside diameter is the same as that of the main or normal wall portion of the tube.

In Fig. 10 there is illustrated an alternative form of expanding apparatus in which a non-rotatable expanding tool 60 is attached to the end of a spindle 61 adapted to be reciprocated by a compressed air or other form of fluid pressure cylinder 62. In Fig. 7 there is shown a tube 65 provided with an end exterior upset 66 which may be either of the normal or relatively thick type, the upset having been thrown to the exterior of the tube by expanding an interior upset in the manner explained with reference to Figs. 6 and 10.

A specific example of tubes requiring exterior end upsets is oil country pump tubing having a 2-inch nominal inside diameter from end to end, a normal wall thickness of 0.19 of an inch, and an upset end wall thickness of 0.30 of an inch, and being 2% inches in outside diameter. Such a tube may be formed from that produced in the first of the above explained examples, the tube when elongated being approximately 30 feet in length and 3 $\frac{1}{8}$  inches in outside diameter, and being provided with normal interior upsets at its ends. After being elongated the tube may be passed through a sink mill to reduce its outside diameter to that required, namely 2% inches. In its passage through the sink mill the length of the tube will be increased in excess of 33 feet, and its wall thickness will be increased somewhat throughout but especially at its ends, resulting in a tube having a normal wall thickness of 0.19 of an inch, an upset end wall thickness of 0.30 of an inch, and an interior diameter of 2 inches throughout its normal wall portion. The upset ends of the tube may then be expanded in the manner explained with reference to either Fig. 6 or 10 to produce the required exterior upsets.

Many of the advantages of my invention are apparent from its foregoing description. In the first place, by its practice upsets are formed on

seamless tubes during their regular course of manufacture, rather than subsequent thereto, and they are formed without any procedural step in addition to those used in the production of seamless tubes having uniform wall thickness from end to end. The result of this is a very substantial saving in the cost of manufacture of upset tubing. In all cases the upsets may be of any desired length and the slopes of transition in wall thickness of the tube from their upsets to their normal thickness walls may be as gradual as desired for any purpose. Thus the upset ends of tubes may be cut back for rethreading, as is frequently done particularly in oil country tubing, and the resistance of the tubes to breakage in their transition sections is greatly increased. Moreover, as the entire procedure involved in the production of upset tubing may be carried out rapidly enough to maintain the entire tube at working temperature during its deformative period, the subsequent cooling of the tube occurs uniformly and as a consequence the tube assumes a normalized condition.

A further advantage of the invention as compared to prior art suggestions that upsets be formed in the course of production of tubing is that the tubes are formed in open passes, by which is meant that they are formed in passes which free the tubes from rather than cause them to be formed tightly upon the mandrels. The result of this is that additional steps are not required to free the formed tubes from the mandrels.

A still further advantage of my invention is that it may be practiced in the production of very thin wall tubing which in its finished form is not provided with upsets. In the hot production of the very thin wall tubing that can be made according to the method disclosed in my aforesaid Patent No. 1,870,209, as, for example,  $\frac{1}{8}$  of an inch in wall thickness, the trailing ends of the tubes sometimes become slightly torn and injure the highly finished surfaces of the guide discs, necessitating the substitution of new discs and the refinishing of those whose peripheral faces have been thus marred. By providing the ends of such thin wall tubing with relatively short upsets, the breaking of their ends may be eliminated. It is obvious that the cost of the scrap loss involved in removing the short upset ends is materially less than the cost incurred by changing and redressing discs whose peripheral faces have been marred by the broken ends of the tubing.

According to the provisions of the patent statutes, I have explained the principle and the mode of operation of my invention, and have illustrated and described the preferred manner of practicing it. However, I desire to have it understood that, within the scope of the appended claims, the invention may be practiced otherwise than specifically disclosed.

I claim:

1. The method of elongating a heated tubular blank and simultaneously reducing its wall principally to a normal and locally to an upset thickness, which comprises cross-rolling the blank continuously from end to end between helically acting reducing rolls and on a longitudinally moving mandrel having a normal-diameter cylindrical portion cooperating with the reducing rolls for determining said normal wall thickness and having a smaller diameter portion for producing said upset wall thickness, and determining the outer diameter of the formed tube by surfaces bearing

on the blank and moving in the direction of its longitudinal movement.

2. The method of elongating a heated tubular blank and simultaneously reducing its wall principally to a normal and locally to an upset thickness, which comprises cross-rolling the blank continuously from end to end between helically acting reducing rolls and on a longitudinally moving mandrel having a normal-diameter cylindrical portion cooperating with the reducing rolls for determining said normal wall thickness and having a smaller diameter portion cooperating with the reducing rolls for determining said upset wall thickness, and determining the outer diameter of the formed tube by surfaces bearing on the blank and moving in the direction of the longitudinal movement of the blank at a speed greater than the longitudinal movement of the blank.

3. The method of elongating a heated tubular blank and simultaneously reducing its wall at its ends to an upset thickness and throughout its intermediate portion to a normal smaller thickness, which comprises cross-rolling the blank continuously from end to end between helically acting reducing rolls and on a longitudinally moving mandrel having an intermediate normal-diameter cylindrical portion cooperating with the reducing rolls for determining said normal wall thickness and having smaller diameter end portions for producing said end upset wall thickness, and determining the outer diameter of the formed tube by surfaces bearing on the blank and moving in the direction of its longitudinal movement.

4. The method of elongating a heated tubular blank and simultaneously reducing its wall principally to a normal and locally to an internal upset thickness, which comprises cross-rolling the blank continuously from end to end on a mandrel moving longitudinally between helically acting reducing rolls and between rotating guide discs, the mandrel having a normal-diameter cylindrical portion for determining said normal wall thickness and having a smaller diameter portion for determining said upset wall thickness, causing the cross-rolls to compress the blank between them and the mandrel at both its normal and smaller diameter portions and to so expand the blank from the mandrel and against the guide discs that the interior circumference of the inwardly upset portion of the blank is greater than the exterior circumference of the normal diameter portion of the mandrel, and causing the guide discs to pull the blank forwardly, whereby the upset thickened wall portion of the blank may freely pass over the normal diameter portion of the mandrel.

5. The method of elongating a heated tubular blank and simultaneously reducing its wall at its ends to an upset thickness and throughout its intermediate portion to a normal smaller thickness, which comprises cross-rolling the blank continuously from end to end on a mandrel moving longitudinally between helically acting reduc-

ing rolls and between rotating guide discs, the mandrel having an intermediate normal-diameter cylindrical portion for determining said normal wall thickness and having smaller diameter end portions for determining said end upset wall thickness, causing the cross-rolls to compress the blank between them and the mandrel at both its end and intermediate portions and to so expand the blank from the mandrel and against the guide discs that the interior circumference of the inwardly upset end portions of the blank is greater than the exterior circumference of the normal diameter intermediate portion of the mandrel, and causing the guide discs to pull the blank forwardly, whereby the upset end portions of the blank may freely pass over the intermediate portion of the mandrel.

6. The method of elongating a heated tubular blank and simultaneously reducing its wall at its ends to an inwardly upset thickness and throughout its intermediate portion to a normal smaller thickness, which comprises cross-rolling the blank continuously from end to end on a mandrel moving longitudinally between helically acting reducing rolls and between rotating guide discs, the mandrel having an intermediate normal diameter portion for determining said normal wall thickness and having smaller diameter end portions for determining said end upset wall thickness, causing the cross-rolls to compress the blank between them and the mandrel at both its end and intermediate portions and to so expand the blank from the mandrel and against the guide discs that the interior circumference of the inwardly upset end portions of the blank is less than the exterior circumference of the normal diameter intermediate portion of the mandrel, causing the guide discs to pull the blank forwardly, and thereafter expanding the inwardly upset ends of the formed tube.

7. The method of elongating a heated tubular blank and simultaneously reducing its wall principally to a normal and at an end to an internal upset thickness, which comprises cross-rolling the blank on a mandrel moving longitudinally between helically acting reducing rolls and between rotating guide discs, the mandrel having a normal-diameter cylindrical portion for determining said normal wall thickness and having a smaller diameter end portion for determining said upset wall thickness, causing the cross-rolls to compress the blank between them and the mandrel at both its normal and smaller diameter portions and to so expand the blank from the mandrel and against the guide discs that the interior circumference of the inwardly upset portion of the blank is smaller than the exterior circumference of the normal diameter portion of the mandrel, and thereafter expanding the inwardly upset portion of the formed tube by moving the normal diameter portion of the mandrel into such upset portion.

SAMUEL E. DIESCHER.